

# UNITED STATES PATENT OFFICE.

FREDERICK M. BECKET, OF NIAGARA FALLS, NEW YORK, ASSIGNOR TO  
ELECTRO METALLURGICAL COMPANY, A CORPORATION OF WEST  
VIRGINIA.

## PROCESS OF REDUCING VANADIUM SULFID.

No. 858,328.

Specification of Letters Patent.

Patented June 25, 1907.

Original application filed March 5, 1907, Serial No. 360,712. Divided and this application filed April 11, 1907. Serial No. 367,619.

To all whom it may concern:

Be it known that I, FREDERICK M. BECKET, a subject of the King of Great Britain, residing at Niagara Falls, in the county of Niagara 5 and State of New York, have invented certain new and useful Improvements in Processes of Reducing Vanadium Sulfid, of which the following is a specification.

In my copending application Serial No. 360,712, filed March 5, 1907, of which the present application is a division, I have described and claimed a process of reducing metallic sulfids, comprising sulfid ores, concentrates, matte or compounds, and specifically the sulfid of molybdenum or molybdenite, by means of silicon or silicon alloys.

The present application relates to a specific embodiment of said process as applied to the reduction of the sulfid or sulfid ores of vanadium, for which the process presents particular advantages as hereinafter set forth.

The usual commercial method of producing vanadium, generally in the form of ferro-vanadium, comprises two steps, vanadinite, 25 roscoelite, or other vanadium ore being first treated in order to obtain therefrom relatively pure vanadium oxid or metallic vanadates, such as those of the alkali or alkaline earth metals or of iron, and such vanadates 30 being then subjected to the reducing action of carbon or aluminium, or to the electrolytic action of the electric current. Sulfid ores of vanadium are roasted to convert the vanadium to the oxidized state, and subsequently 35 treated for the extraction of vanadium oxid or production of metallic vanadates.

I have found that commercially pure vanadium may be produced by smelting in an electric furnace a mixture of vanadium sulfid 40 and silicon or an alloy of silicon, the silicon being preferably employed in substantially the proportions required to combine with the sulfur of the sulfid or ore, the equation assuming the production of silicon sulfid,  $SiS_2$ . 45 I have also found that commercially pure alloys of vanadium may be produced by smelting in an electric furnace a mixture of vanadium sulfid with a silicon alloy, such as ferro-silicon or nickel-silicon, the alloy being preferably used in approximately the proportions required to supply sufficient silicon to 50 unite with the sulfur of the sulfid, or sulfid ore.

In operation the sulfid, and a silicon-bear-

ing reducing agent, comprising either silicon 55 or a silicon alloy, both in a moderately fine state of subdivision, are smelted in any suitable electric furnace, which should preferably, in case a product low in carbon is required, be provided with a hearth or lining of material other than carbon. It is not essential that the proportion of silicon to sulfur should be precisely that indicated by theory, for in case a product very low in silicon is required 60 the sulfid should preferably be used in excess of such proportion; whereas if a certain proportion of silicon is permissible in the product an excess of the silicon or silicon-bearing reducing agent may be used. The operation is preferably rendered continuous 65 in character by adding fresh portions of the charge from time to time and withdrawing the product as desired.

By smelting the charge in a close chamber and protecting the products from oxidizing 75 influences the sulfid of silicon may be collected, but in open smelting furnaces both of the constituent elements of the sulfid unite with oxygen, yielding silica in a state of minute subdivision and sulfur dioxide; these 80 products may be collected and utilized as desired.

In the production of the alloys of vanadium with iron, nickel and the like, I may incorporate iron, nickel, or other metal with 85 the charge prepared for the reduction of vanadium, or I may introduce the desired proportions of these metals into the furnace at any time during the operation; or the metals, iron or nickel, for example, may be reduced 90 from their compounds simultaneously with the reduction of the vanadium without interfering with the process.

By the use of this direct process it is not only possible to omit the usual roasting and 95 other preliminary operations on sulfid ores, but to produce commercially pure metals or alloys without the previous treatments generally employed for the removal of silicious material, with which these ores are associated. For example, from the important Peruvian ores of vanadium, in which the vanadium exists as a sulfid or mixture of sulfids associated with a considerable proportion of silicious matter, I have found that commercially 100 pure ferro-vanadium may be produced by direct smelting in presence of iron or ores of iron with silicon or silicon alloys.

I claim:

1. The process of reducing vanadium sulfid which consists in reacting thereon with silicon.
- 5 2. The process of reducing vanadium sulfid which consists in reacting thereon with a silicon alloy.
3. The process of reducing vanadium sulfid which consists in reacting thereon with ferro-silicon.
- 10 4. The process of reducing vanadium sulfid which consists in reacting thereon with silicon in substantially the proportion required to unite with the sulfur of the sulfid.
5. The process of reducing vanadium sulfid

which consists in reacting thereon with ferro-silicon in substantially the proportion required to unite with the sulfur of the sulfid.

6. The continuous process of reducing vanadium sulfid which consists in smelting a mixture of said sulfid and silicon, adding fresh portions of the charge, and withdrawing the product as desired.

In testimony whereof, I affix my signature in presence of two witnesses.

FREDERICK M. BECKET.

Witnesses:

J. W. H. RANDALL,  
CARLETON F. BROWN